



soluble in alcohol, benzene and kerosene and had the formula:



where  $\text{R}_1$ ,  $\text{R}_2$  and  $\text{R}_3$  are an aliphatic long chain present in castor oil fatty acid groups.

These castor oil fatty acids are derived from the still bottoms resulting from castor oil distillation procedures.  $\text{R}_3\text{COOH}$  is a salt forming group attached to the tertiary nitrogen.

#### EXAMPLE 4

One mol of N-hydroxyethylpiperazine and three mols of tall oil fatty acids containing 33% rosin acids was reacted at 350°-375° F. until two mols of water was collected in the water trap.

The resulting compound was a viscous reddish-brown liquid having the following formula:



where  $\text{R}_1$  and  $\text{R}_2$  are groups containing an aliphatic long chain present in tall oil fatty acid groups.

In this reaction, the  $\text{R}_1$  and  $\text{R}_2$  of the oleic and linoleic acids first combine in mixture with the terminal reactive group and with the abietic acid finally combining with the tertiary amine to form a salt. The  $\text{R}_1$  acid grouping combines with the secondary nitrogen to form an amide. The  $\text{R}_2$  acid group forms an ester with the hydroxy groups.  $\text{R}_1$  and  $\text{R}_2$  related to the same oleic-linoleic compositions.

The compounds of Examples 3 and 4 include an additive consisting of a high molecular weight fatty acid compound having 14 to 22 carbon atoms which fatty acid has been condensed with a piperazine ring compound and having at least two aliphatic side chains attached to at least one nitrogen of the ring, one side chain including a fatty acid residue having 14 to 22 carbon atoms another side chain polymethylene linkage having 2 or 3 carbon atoms and terminating in an amino group carrying a fatty acid residue having 14 to 22 carbon atoms.

Specifically they have the formula



where  $\text{W}$  is a fatty acid residue containing 14 to 22 carbon atoms and  $\text{Z}$  is a fatty acid amide with a fatty acid containing 14 to 22 carbon atoms and  $n$  represents a numeral 2 or 3.

Or more specifically the formulae



where  $\text{R}$  stands for an aliphatic long chain present in tall oil fatty acid group.

Or



where  $\text{R}_1$ ,  $\text{R}_2$  and  $\text{R}_3$  are aliphatic long chains present in fatty acid groups containing 12 to 22 carbon atoms.



where  $\text{R}_1$  and  $\text{R}_2$  are respectively groups containing aliphatic long chains present in tall oil fatty acid groups.

The above derivatives were evaluated for their wetting and anti-stripping properties by incorporating 1% in MC-3 asphalt by the method as outlined below.

Ninety-nine grams samples of MC-3 liquid asphalt was thoroughly blended with one gram of asphalt additive as prepared in Examples 1 to 4 in a half pint friction-top can. The containers were placed in an oven maintained at a temperature of 325° F. for 72 hours, at the end of which period of time, the samples were removed and cooled to 175° F.

At the same time 100 grams of MC-3 asphalt without additive was heated for the same period under the same conditions to give a blank run.

#### Wet Coating Test

One hundred gram samples of  $\frac{3}{8}$ " size reference aggregate were weighed into 8-ounce containers. Then the samples were subjected to wet coating and stripping tests.

Two grams of distilled water was weighed into each container and mixed with the aggregate until thoroughly wet. Six grams of the prepared MC-3 asphalt prepared with the additive according to any one of Examples 1 to 4 was added to the wetted aggregate and thoroughly mixed for five minutes.

At least 95% of the aggregate surfaces was coated as evaluated by visual inspection.

The blank of MC-3 asphalt failed the test.

#### Stripping Test

The coated aggregate from the "Wet Coating Test" was formed into a compact mass one inch thick and cured for one hour at 140° F.

The cured mixes were then immersed in distilled water at room temperature and allowed to remain for 18 hours. At least 95% of the aggregate surfaces was coated at the end of the immersion period.

The blank of MC-3 asphalt failed the test with zero coating.

The following are the results of 72 hour heat stability test at 325° F.

TABLE I.—WET COATING TEST  
[Percent coated]

| MC-3 Asphalt plus Additive | Massachusetts Rhyolite | New York Granite | Ohio Silica | Virginia Limestone |
|----------------------------|------------------------|------------------|-------------|--------------------|
| Example 1.....             | 96                     | 95               | 100         | 90                 |
| Example 2.....             | 95                     | 100              | 100         | 100                |
| Example 3.....             | 100                    | 100              | 100         | 95                 |
| Example 4.....             | 100                    | 100              | 100         | 100                |

TABLE II.—EIGHTEEN HOUR WATER IMMERSION TEST  
[Percent coated aggregate]

| MC-3 Asphalt plus Additive | Massachusetts Rhyolite | New York Granite | Ohio Silica | Virginia Limestone |
|----------------------------|------------------------|------------------|-------------|--------------------|
| Example 1.....             | 90                     | 95               | 95          | 90                 |
| Example 2.....             | 90                     | 100              | 90          | 90                 |
| Example 3.....             | 95                     | 100              | 90          | 90                 |
| Example 4.....             | 95                     | 95               | 90          | 100                |

The additive compounds are added in amounts ranging from  $\frac{1}{4}\%$  to 30% of the weight of the asphalt or bituminous material or tar. Preferably the range is  $\frac{1}{2}$  to  $\frac{1}{2}\%$  by weight of the asphalt.

Usually, the additive is included in asphalt compositions such as medium cure, cutback with 30% kerosene,

